

## UNITED STATES PATENT OFFICE

2,441,179

## METHOD OF REMOVING METAL FROM THE SURFACE OF BLOOMS AND THE LIKE

James L. Anderson, Closter, N. J., assignor to Air Reduction Company, Incorporated, a corporation of New York

No Drawing. Application July 21, 1945,  
Serial No. 606,477

5 Claims. (Cl. 148—9)

1

This invention relates to the thermo-chemical removal of metal from the surface of blooms, billets, slabs and other metal bodies. This operation is sometimes referred to as scarfing.

When blooms, billets and other rolled metal bodies come from the rolling mills they usually have surface imperfections and adhering oxide and scale. Scarfing is performed on the metal bodies to remove a layer of the surface metal and thereby remove the surface imperfections before the final rolling operations. A common way of performing the scarfing operation is to project against the surface to be scarfed, while the metal is at kindling temperature, oxygen streams delivered by a burner block, and causing relative movement of the surface and the oxygen streams so that the oxygen progressively removes the surface metal. Before the scarfing operation can be started the portion of the surface where the scarfing is to be initiated must be conditioned by removing the oxide and scale. This is usually accomplished by the use of heating flames which issue from the burner and which are projected against the surface to fuse the oxide and scale and thereby initiate the scarfing operation when the scarfing oxygen is turned on. Heretofore some delay has been experienced in starting the scarfing operation because of the time required to fuse the oxide and scale. Because of the insulating effect of the oxide and scale, and because of the tendency of the oxide to build up when using heating flames of the usual character, it has been necessary to heat the oxide and scale for a period ranging anywhere from 13 to 20 seconds before the scarfing operating could be started.

The principal object of this invention is to so modify the usual method of removing metal from the surface of metal bodies having adhering oxide and scale that the time required for the heating and surface-conditioning step is greatly reduced or entirely eliminated.

According to the invention the heating of the surface where the scarfing is to be initiated is performed by the use of oxyacetylene flame jets which have a reducing action. The supply of oxygen and acetylene to the flame jets is adjusted so that there is an excess of acetylene to produce reducing flames having a so-called acetylene feather which is preferably sufficiently long to extend to the surface to be scarfed.

The film or layer of oxide on the surface of a hot bloom or billet is usually at a temperature of 2000° F. or higher and the reducing flames act instantly on it and change the oxide to metallic

2

iron. The film of oxide may be changed into particles of iron which coalesce into molten globules, or it may be changed into a film of metallic iron which is caused to form into molten globules by surface tension. In either case when the scarfing oxygen is turned on, the globules of metallic iron burn and create a temperature considerably above the temperature of the hot bloom and cause the surface metal of the bloom to ignite immediately. They act like a number of starting rods producing instantaneous action. As the globules ignite they are forcibly pressed against the surface of the bloom by the scarfing oxygen streams so that the ignition of the surface metal of the bloom and the globules is simultaneous. The bloom being at a temperature of approximately 2000° F. is well above the critical ignition point of the steel, and when the oxide is reduced to globules of metallic iron having the action above described, the surface metal of the bloom is ready for instant ignition without pre-heating. It will thus be seen that almost instantly after the reducing flames are projected against the layer of oxide and scale the scarfing oxygen can be turned on and the scarfing operation started, whereby the reduction of the oxide takes place at a temperature below its fusion point and the period of time heretofore required for the flames to fuse the oxide and scale is eliminated. Preferably, the reducing character of the flames is maintained during the entire scarfing operation.

Oxyacetylene flames adjusted so that they are reducing in character produce a less intense heat, 35 of course, than neutral flames. For this reason, and because of the presence of the oxide and scale on the surface to be scarfed, one would naturally be led away from the use of reducing flames for the usual preliminary heating operation. It 40 would be expected that they are either not hot enough to be useful at all for such operation, or would unduly lengthen the time required for its performance. Contrary to these expectations I have discovered that despite their less heat intensity reducing flames actually lessen the time required for conditioning the surface to be scarfed to such an extent that when scarfing hot blooms or billets the scarfing can be started instantly after the flames are brought into contact with the 50 work surface.

While the method is particularly suited for the scarfing of hot blooms, billets, slabs and the like, and has been described in that connection, it may also be used for scarfing cold work-pieces 55 having adhering oxide and scale. In this case,

however, it may be necessary to wait a few seconds after bringing the flames into contact with the layer of oxide and scale before the scarfing oxygen is turned on, but not nearly so long as would be necessary if the flames were of the usual neutral character.

I claim:

1. The method of desurfacing blooms, billets, slabs, and other metal bodies having adherent oxide and scale, which comprises reducing the oxide on the surface of the metal body at the place where the desurfacing operation is to begin to molten metallic iron by projecting reducing flames against the surface at that place, and, after the oxide at that place on the surface has been reduced to molten metallic iron, and while it still is in such molten state, projecting an oxygen stream against that place on the surface, and then causing relative movement of the surface and oxygen stream at such relative rate as to remove the surface only of the body.

2. The method of desurfacing blooms, billets, slabs, and other metal bodies having adherent oxide and scale, which comprises reducing the oxide on the surface of the metal body at the place where the desurfacing operation is to begin to molten metallic iron by projecting flames fed by a mixture of oxygen and acetylene in which there is an excess of acetylene against the surface at that place, and, after the oxide at that place on the surface has been reduced to molten metallic iron and while it still is in such molten state, projecting an oxygen stream against that place on the surface, and then causing relative movement of the surface and oxygen stream at such relative rate as to remove the surface only of the object.

3. The improvement in the starting of the desurfacing of blooms, billets, slabs and other metal bodies having adherent oxide and scale by projecting an oxygen stream against a heated surface thereof and relatively moving the surface and oxygen stream to progressively remove the surface only of the body which comprises heating the surface at that place where the desurfacing operation is to begin to a temperature at which the adherent oxide will reduce to molten metal when in contact with a reducing gas, but below the fusion point of the oxide, and projecting onto the thus heated surface a reducing gas to substantially instantly reduce the oxide to molten metallic iron, and immediately thereafter projecting the oxygen stream against the surface at that place and proceeding with the desurfacing

operation, whereby the reduction of the oxide takes place at a temperature below its fusion point and without preliminary fusing thereof.

4. The improvement in the starting of the desurfacing of blooms, billets, slabs and other metal bodies having adherent oxide and scale by projecting an oxygen stream against a heated surface thereof and relatively moving the surface and oxygen stream to progressively remove the surface only of the body which comprises heating the surface at that place where the desurfacing operation is to begin to a temperature at which the adherent oxide will reduce to molten metal when in contact with a reducing gas, but below the fusion point of the oxide, and projecting onto the thus heated surface a flame fed by a mixture of oxygen and acetylene in which there is an excess of acetylene to substantially instantly reduce the oxide to molten metallic iron, and immediately thereafter projecting the oxygen stream against the surface at that place and proceeding with the desurfacing operation, whereby the reduction of the oxide takes place at a temperature below its fusion point and without preliminary fusing thereof.

5. In the method of desurfacing hot blooms, billets, slabs, and other metal bodies having adherent oxide and scale by projecting an oxygen stream against the surface while the metal is at a kindling temperature and relatively moving the surface and oxygen stream to progressively remove the surface metal, the improvement in starting the operation which comprises first reducing the oxide on the portion of the surface on which the oxygen stream initially is to be projected to molten metallic iron by projecting against such portion of the surface flames which are reducing in character, and then projecting the oxygen stream against the portion of such surface containing the molten metallic iron.

JAMES L. ANDERSON.

#### REFERENCES CITED

The following references are of record in the file of this patent:

#### UNITED STATES PATENTS

| Number       | Name        | Date         |
|--------------|-------------|--------------|
| 1,957,351    | Oldham      | May 1, 1934  |
| 50 2,210,402 | Gaines, Jr. | Aug. 6, 1940 |

#### OTHER REFERENCES

Metals Handbook, 1936 edition, page 138, (pub. by American Society for Metals, Cleveland, Ohio).